

April 6, 1965

M. MAESER

3,176,333

METHODS OF CONDITIONING SHOE UPPERS

Filed Sept. 17, 1963

2 Sheets-Sheet 1



Fig.1

Fig.2



Fig.3



Inventor

Mich Maeser

By his Attorney

*W. L. Maeser*

April 6, 1965

M. MAESER

3,176,333

METHODS OF CONDITIONING SHOE UPPERS

Filed Sept. 17, 1963

2 Sheets-Sheet 2



1

3,176,333

METHODS OF CONDITIONING SHOE UPPERS  
Mieth Maeser, Beverly, Mass., assignor to United Shoe  
Machinery Corporation, Flemington, N.J., a corpora-  
tion of New Jersey  
Filed Sept. 17, 1963, Ser. No. 309,417  
23 Claims. (Cl. 12—142)

This invention relates to a process of conditioning leather and, more particularly, to a method of conditioning upper leather comprising an improved method of mulling prior to lasting and a novel method of setting subsequent to lasting, this application being a continuation-in-part of an application Serial No. 253,833, filed January 25, 1963, in the name of Mieth Maeser, now abandoned.

The conditioning of upper leather is a problem which has plagued the shoemaking industry throughout the years. Numerous attempts have been made to solve the problem but until the subject invention no solution was forthcoming which improved the characteristics of leather important to lasting to the maximum degree possible and also accomplished the set required in a minimum period of time. Proper conditioning of leather is of paramount importance not only to the quality of the finished shoe but also to the workability of the leather during the manufacture thereof. In order to facilitate the lasting of a shoe, the flexibility and stretchability of the upper leather must be increased. Accordingly, the value of a method of conditioning upper leather prior to lasting is largely determined by the degree to which it increases the above-noted characteristics. However, the lasting of a shoe upper involves principally the stretching and compressing of the leather and, therefore, the characteristic of stretchability takes precedence in selecting the method of conditioning. Thus, the problem of prelasting conditioning is to devise a method of mulling which attains maximum stretchability and also increases the flexibility a maximum amount based upon a stretchability increase.

The setting of a shoe upper subsequent to lasting affects the quality, durability, wearability and appearance of the finished shoe. The moisture imparted to the upper leather during prelasting conditioning must be removed in sufficient quantity to place the leather in normal condition and the leather must be set in the configuration imposed by the last. The quality and degree of set attained determines the length of time the shoe will remain in the configuration originally imparted thereto. The principal end to be accomplished in the setting of a shoe upper is the relief of any stresses existing within the leather prior to lasting and those induced by lasting thereby to permit the shoe to assume the configuration desired without contrary residual stresses or memory. The appearance of the shoe is also affected by the shrinkage of the upper leather on the last. A method of setting should permit that amount of shrinkage necessary to impose the last configuration into the leather and eliminate wrinkles therefrom but must not result in excessive shrinkage whereby the leather is damaged or marred.

A further problem which pervades conditioning of leather in the manufacture of shoes is the economic aspects of the conditioning process. The duration of the conditioning operations determines the number of lasts the manufacturer must employ. A conditioning method which markedly shortens the period of time a shoe must remain on the last enables a manufacturer to reduce the number of lasts being utilized thereby diminishing the overall cost of making the shoe. Further, proper prelasting conditioning facilitates an increase in the speed and efficiency of the lasting operations and, thus, considerable cost savings.

2

In view of the foregoing, an object of the present invention is to provide a method of conditioning upper leather which places the leather in a condition of maximum stretchability and correlated flexibility prior to the lasting operations and which attains optimum set of the upper leather after lasting thereof has been completed.

A further object of this invention is the attainment of the above-noted ends in a minimum period of time consistent with quality shoe manufacturing standards.

To this end and in accordance with a feature of the present invention, there is provided a method of shoemaking comprising subjecting a leather upper to a humidified atmosphere to distribute water uniformly throughout the upper leather, heating the leather upper in high temperature moist air, lasting the leather upper while it is moist and at a high temperature, heating the lasted upper in a moist atmosphere, and drying the lasted upper in a dry atmosphere.

An alternative species of the above method is also provided wherein the heating and drying completed subsequent to lasting are performed in a single high temperature moist atmosphere.

The above and other features of the invention will now be described, the accompanying drawings being included to aid in the delineation thereof.

FIG. 1 is a cross-sectional view of a piece of leather;  
FIG. 2 is a graph illustrating the effect of moisture and temperature on the stiffness of leather;

FIG. 3 is a graph illustrating the effect of moisture and temperature on the distortion at grain burst, and, thus, on the stretchability of the grain;

FIG. 4 is a graph illustrating the effect of moisture and temperature on the distortion at total burst and, thus, on the stretchability of leather; and

FIG. 5 is a graph illustrating the effect of moisture and temperature on the permanent set.

In order to appreciate the advantages of the present invention an analysis of certain characteristics of leather must be made and the effect thereof on conditioning weighed. As illustrated in FIG. 1, a leather skin comprises a grain area 10, a corium 12, and a mucoid layer 14. The mucoid layer 14 is primarily a bonding between the grain and the corium and is of little significance to the structural properties of leather. The grain area 10 has approximately one half the tensile strength of the corium 12. Therefore, when a leather upper is overworked the grain layer ruptures first. However, in the normal leather cross-section the greatest portion is composed of corium fibers and, thus, this area is of primary significance in conditioning the leather. As noted above, the lasting of a leather upper involves principally the stretching and compressing of the fibrils of the leather. The flexibility of the leather is significant in that it must be increased to permit that flexing resulting from lasting over the feather line and to prevent cracking of the grain area but it is of secondary importance to an increase in stretchability.

The graphs of FIGS. 2-4 illustrate the effects of moisture upon leather. Immediately upon the application of moisture to the surface fibers of the leather, the flexibility of the grain is increased and, therefore, the flexibility of the entire member. When the moisture is confined primarily to the grain area, stretchability of the grain area per se is increased. However, this increase in the stretchability of the grain area is of negligible significance to the overall workability of the leather as a result of the condition of the corium. This is equally true when moisture is applied and confined to the grain and the outer surface of the corium disposed from the grain as the effect on the total corium area is minimal. If the total moisture content of the leather upper remains approxi-

mately constant, maximum flexibility exists when the moisture is concentrated in the outside fibers which include the grain area since the grain area is the outer fiber area in the bending beam theory and, further, due to the inherent physical properties thereof. However, as the moisture disperses through the leather the stretchability is increased due to the permeation of the corium by the moisture. Thus, an end to be attained by a method of conditioning prior to lasting is the distribution of moisture throughout the leather and sufficient concentration of moisture in the grain area to permit flexing during the lasting operations.

The application of heat has a marked influence on the mulling of leather, as illustrated in FIGS. 2-4. Heat lowers the viscosity and surface tension of liquid and enables it to penetrate the surface more readily. Further, the heat acts to soften the moist fibrils of the leather thereby to increase the workability thereof. Thus, heat is an important adjunct of moisture in the conditioning of leather.

As stated above, the primary objective in the setting of leather subsequent to lasting is the relief of residual stresses and memory and the imposition of stresses and memory which tend to retain the upper leather in the configuration imparted thereto by the lasting operations. The relative size of the corium therefore requires that a conditioning method relieve the residual stresses and memory therein if the method is successfully to set the upper leather in the desired shape. The combination of moisture and heat have a stress relieving effect on leather. The graphs of FIG. 5 illustrate the influence of moisture and heat on the setting of leather. With sufficient moisture present in the leather heat is able to reach the moisture and soften the fat liquors and fibers of the grain and corium thereby to allow maximum movement of the fibers. As a result, the internal stresses caused by residual tanning effects, finishing, and pulling and lasting are released and the residual memory dissipated thereby "normalizing" the fibers of the grain and corium and preparing the leather for the imposition of retaining stresses and memory. When the residual stresses have been relieved, as defined above, the upper can be set by heating to remove excessive moisture and impose retaining stresses and memory. The drying also serves to shrink the upper whereby the upper is subjected to the configuration of the last. The grain area, due to its relative size and position, is subjected to a greater amount of heat and, accordingly, shrinks more than other portions of the leather thereby resulting in the elimination of wrinkles in the surface thereof. The time permitted for drying is important not only with respect to the economic production of shoes but also in that it must be of sufficient duration to permit the negation of creep within the upper. A method which attempts to solve the problem of rapid drying by applying moisture only to the surface areas or grain of the leather and removing the same before it permeates the corium, fails to take advantage of the stretchability characteristics of the corium and, further, has no effect on the stresses and memory of the corium.

In the application of the method of the subject invention a leather upper is initially mulled in a humidified atmosphere to distribute water uniformly throughout the grain and corium of the upper leather. The normal moisture content of leather is between 8% and 11%. The object of the mulling operation is to increase the moisture content to 15% to 25%. This operation insures that the leather will be of maximum stretchability prior to the lasting operations. After the mulling operation is completed, the leather upper is heated in a high temperature moist atmosphere. The temperature of the moist atmosphere should be between 140° F. and 300° F. but preferably would be in the 250° F. to 300° F. range. This step in the method is actually a heating operation which is accomplished without drying the leather. The humidity level must be maintained at a

magnitude sufficient to insure at least moisture equilibrium between the atmosphere and the leather thereby to prevent drying of the leather. This is accomplished by maintaining the dew point of the atmosphere above the temperature of the upper leather. The result of this step is to precipitate a film of water on the surface or grain of the leather. The presence of the upper in the heated atmosphere condenses this water film and the heat of condensation results in rapid heating of the upper. Further, since a moist surface will pick up more heat than a dry surface the rate of heating of the upper leather will be increased until the surface of the grain is dry. The result of the above is that water is distributed throughout the leather, moisture is concentrated in the grain area below the surface thereof and the leather is rapidly brought to the desired temperature level.

After the lasting operations have been completed, the shoe is again heated in a high temperature moist atmosphere. The temperature of the atmosphere should preferably be above the boiling point in the 220° F. to 375° F. range and the dew point of the atmosphere above the temperature of the shoe. As explained above, this facilitates rapid heating of the upper leather without removing the moisture previously imparted thereto thereby providing the combination of moisture and heat required for stress relief. Further, this heating step is accomplished without adding an appreciable amount of moisture as the 15 to 25% moisture content already in the leather upper represents substantially the maximum saturation which can be obtained under the conditions involved. This step "normalizes" the leather thereby relieving the residual stresses referred to above. The temperature of the atmosphere should be regulated for a particular leather to insure that the grain of the leather is not lifted or made rough. The purpose of this step is to heat the leather, not to dry it.

The final step in the method of this invention is to draw the moisture out of the leather to set the upper in the configuration imparted by the last and to lock the leather in the new shape by heating in a dry atmosphere, preferably at a temperature above the boiling point of water. The result of this last operation is to impart a new memory to the leather which ties the fibers in the new shape imposed by the last. The combination of temperature and time required to dry the leather should be such that the excess moisture is completely removed, the creep tendencies dissipated, the wrinkles chased and memory imposed. The end accomplished by this operation can be attained by merely permitting exposure of the upper to the surrounding atmosphere for a sufficient period of time. However, heating thereof in a dry atmosphere reduces the time required for setting and results in better set.

The two steps of the above described method performed subsequent to lasting may, in the alternative, be combined into a unitary step employing a single atmosphere to both heat and dry the lasted upper. This is accomplished by the use of a high temperature moist atmosphere the dew point and temperature of which are controlled such that, for a given exposure interval, the temperature of the exposed upper is elevated from a level below the dew point to a level thereabove. In the practice of this alternative species, an upper is introduced to a humidified atmosphere having a dew point above the initial temperature of the upper. Thus, initially during exposure of the upper, the temperature thereof is raised without withdrawing moisture therefrom. The exposure interval is regulated such that the temperature of the upper is raised above the dew point of the atmosphere thereby resulting in moisture removal from the upper thereafter. Ergo, a single humidified atmosphere is utilized to heat the moist upper thereby to relieve the residual stresses therein and to dry the upper thereby to set the upper in the configuration imparted by the last.

Having thus described my invention, what I claim as

new and desire to secure by Letters Patent of the United States is:

1. The method of setting a moistened shoe upper on a last subsequent to completion of all the lasting operations to impart to said upper a permanent reproduction of the shape of the last comprising heating the upper in a moist atmosphere while the upper is on the last thereby to heat the moisture and fat liquors in the upper to soften the fibers of the grain and of the corium to relieve stresses in said fibers without adding an appreciable amount of moisture to the upper and subsequently drying the upper while on the last in a high temperature dry atmosphere to remove moisture therefrom and thereby impart stresses to the fibers of the grain and of the corium of the upper which thereafter produce a permanent reproduction of the shape of the last.

2. The method of shoemaking comprising subjecting a leather upper to a humidified atmosphere to raise the moisture content thereof to 15% to 25% uniformly distributed throughout the upper leather, heating the upper leather in 140° F. to 300° F. moist air, said moist air having a dew point above the temperature of the upper leather, lasting the leather upper while said upper is at a high temperature and moist, heating the lasted upper in a moist atmosphere, said moist atmosphere being in the temperature range of 220° F. to 375° F. and having a dew point above the temperature of the upper leather, and drying the lasted upper in a high-temperature dry atmosphere.

3. The method of shoemaking comprising subjecting a leather upper to a humidified atmosphere to raise the moisture content thereof to 15% to 25% uniformly distributed throughout the upper leather, heating the upper leather in 140° F. to 300° F. moist air, lasting the leather upper while said upper is at a high temperature and moist, heating the lasted upper in a moist atmosphere, said moist atmosphere being in the temperature range of 220° F. to 375° F., and drying the lasted upper in a high-temperature dry atmosphere.

4. The method of shoemaking comprising subjecting a leather upper to a humidified atmosphere to raise the moisture content thereof to 15% to 25% uniformly distributed throughout the upper leather, heating the upper leather in high-temperature moist air, said moist air having a dew point above the temperature of the upper leather, lasting the leather upper while said upper is at a high temperature and moist, heating the lasted upper in a moist atmosphere, said moist atmosphere having a dew point above the temperature of the upper leather, and drying the lasted upper in a high-temperature dry atmosphere.

5. The method of shoemaking comprising subjecting a leather upper to a humidified atmosphere to distribute water uniformly throughout the upper leather, heating the upper leather in high temperature moist air, said moist air being in the temperature range of 140° F. to 300° F. and having a dew point above the temperature of the upper leather, and lasting the leather upper while said upper is still moist and at a high temperature.

6. The method of conditioning upper leather subsequent to lasting comprising heating the upper in a moist atmosphere, said atmosphere being in the temperature range of 220° F. to 375° F. and having a dew point above the temperature of said upper, and drying the upper in a high-temperature dry atmosphere.

7. The method of shoemaking comprising subjecting a leather upper to a humidified atmosphere to raise the moisture content thereof to 15% to 25% uniformly distributed throughout the upper leather, heating the upper leather in high-temperature moist air, said moist air being in the temperature range of 140° F. to 300° F., and lasting the leather upper while said upper is still moist and at a high temperature.

8. The method of conditioning upper leather subsequent to lasting comprising heating the upper in a moist atmosphere, said atmosphere being in the temperature

range of 220° F. to 375° F., and drying the upper in a high-temperature dry atmosphere.

9. The method of shoemaking comprising subjecting a leather upper to a humidified atmosphere to distribute water uniformly throughout the upper leather, heating the upper leather in high-temperature moist air, said moist air having a dew point above the temperature of the upper leather, and lasting the leather upper while said upper is still moist and at a high temperature.

10. The method of setting a moistened shoe upper on a last subsequent to completion of all the lasting operations to impart to said upper a permanent reproduction of the shape of the last comprising heating the upper in a moist atmosphere while the upper is on the last thereby to heat the moisture and fat liquors in the upper to soften the fibers of the grain and of the corium to relieve stresses in said fibers without adding an appreciable amount of moisture to the upper, said atmosphere having a dew point above the temperature of said upper, and subsequently

15 drying the upper while on the last in a high temperature dry atmosphere to remove moisture therefrom and thereby impart stresses to the fibers of the grain and of the corium of the upper which thereafter produce a permanent reproduction of the shape of the last.

20 11. The method of shoemaking comprising subjecting a leather upper to a humidified atmosphere to distribute water throughout the upper leather, heating the upper leather in high-temperature moist air, said moist air being in the temperature range of 140° F. to 300° F., lasting the leather upper while it is still moist and at a high temperature, and heating the lasted upper in a moist atmosphere, said moist atmosphere being in the temperature range of 220° F. to 375° F.

25 12. The method of shoemaking comprising subjecting a leather upper to a humidified atmosphere to distribute water throughout the upper leather, lasting the leather upper while said upper is moist, and heating the lasted upper in a moist atmosphere, said moist atmosphere being in the temperature range of 220° F. to 375° F.

30 13. The method of shoemaking comprising subjecting a leather upper to a humidified atmosphere to distribute water throughout the upper leather, heating the upper leather in high-temperature moist air, said moist air being in the temperature range of 140° F. to 300° F. and having a dew point above the temperature of the upper leather,

35 45 lasting the leather upper while it is still moist and at a high temperature, and heating the lasted upper in a moist atmosphere, said moist atmosphere being in the temperature range of 220° F. to 375° F. and having a dew point above the temperature of the upper leather.

50 55 14. The method of shoemaking comprising subjecting a leather upper to a humidified atmosphere to distribute water throughout the upper leather, lasting the leather upper while said upper is moist, and heating the lasted upper in a moist atmosphere, said moist atmosphere being in the temperature range of 220° F. to 375° F. and having a dew point above the temperature of the upper leather.

60 65 15. The method of shoemaking comprising subjecting a leather upper to a humidified atmosphere to add water throughout the upper leather, heating the upper leather in high-temperature moist air, said moist air having a dew point above the temperature of the upper leather, lasting the leather upper while it is still moist and at a high temperature, and heating the lasted upper in a moist atmosphere, said moist atmosphere having a dew point above the temperature of the upper leather.

70 75 16. The method of shoemaking comprising subjecting a leather upper to a humidified atmosphere to add water throughout the upper leather, lasting the leather upper while said upper is moist, and heating the lasted upper in a moist atmosphere, said moist atmosphere having a dew point above the temperature of the upper leather.

17. The method of shoemaking comprising subjecting a leather upper to a humidified atmosphere to raise the moisture content thereof to 15% to 25% uniformly

distributed throughout the upper leather, lasting the upper while said upper is moist, heating the lasted upper in a moist atmosphere to relieve the stresses therein, and drying the lasted upper in a high-temperature dry atmosphere.

18. The method of setting a moistened leather shoe upper on a last subsequent to completion of all the lasting operations to impart to said upper a permanent reproduction of the shape of the last comprising exposing the upper to a high-temperature moist atmosphere having a dew point above the initial temperature of the upper thereby to heat the moisture and fat liquors in the upper to soften the fibers of the grain and of the corium to relieve stresses in said fibers without adding an appreciable amount of moisture to the upper and maintaining the upper exposed to said atmosphere for a period sufficient to raise the temperature of the upper above the dew point of the atmosphere thereby to dry the upper to impart stresses to the fibers of the grain and of the corium of the upper which thereafter produce a permanent reproduction of the shape of the last.

19. The method of setting a moistened shoe upper on a last subsequent to completion of all the lasting operations to impart to said upper a permanent reproduction of the shape of the last comprising heating the upper in a high-temperature moist atmosphere while the upper is on the last thereby to heat the moisture and the fat liquors to soften the fibers of the grain and of the corium and to relieve stresses in said fibers without adding an appreciable amount of moisture to the upper, said atmosphere having a dew point above the initial temperature of the upper, maintaining the upper exposed to said moisture for a period sufficient to raise the temperature of the upper above the dew point of the atmosphere, and subsequently drying the upper while on the last by exposure to said atmosphere subsequent to the reversal of the relative magnitude of said dew point and temperature thereby to impart stresses to the fibers of the grain and of the corium of the upper which thereafter produce a permanent reproduction of the shape of the last.

20. The method of shoemaking comprising subjecting a leather upper to a humidified atmosphere to add moisture throughout the upper, lasting the upper while said upper is moist, heating the upper in a high temperature moist atmosphere having a dew point above the temperature of the upper prior to exposure thereto for a period sufficient to raise the temperature of the upper above the dew point of the atmosphere, and thereafter drying the upper in said atmosphere.

21. The method of shoemaking comprising subjecting a leather upper to a humidified atmosphere to add moisture throughout the upper, heating the upper in a high temperature moist atmosphere, lasting the upper while said upper is at a high temperature and moist, heating the upper in a high temperature moist atmosphere, said atmosphere having a dew point above the temperature of the upper prior to exposure to said atmosphere, maintaining the upper exposed to said atmosphere for a period sufficient to raise the temperature of the upper above the dew point of the atmosphere, and drying the upper by exposure to said atmosphere subsequent to the reversal of the relative magnitude of said dew point and temperature.

22. The method of setting a moistened shoe upper on a last subsequent to completion of all the lasting operations to impart to said upper a permanent reproduction of the shape of the last comprising heating the upper in a high temperature moist atmosphere having a dew point above the temperature of the atmosphere prior to exposure thereto for a period sufficient to raise the temperature of the upper above the dew point of the atmosphere thereby to heat the moisture and fat liquors in the upper to soften the fibers of the grain and of the corium to relieve stresses in said fibers without adding an appreciable amount of moisture to the upper, said atmosphere being in the temperature range of 200° F. to 300° F., and thereafter drying the upper in said atmosphere to impart stresses to the fibers of the grain and of the corium of the upper which thereafter produces a permanent reproduction of the shape of the last.

23. The method of shoemaking comprising subjecting a leather upper to a humidified atmosphere to raise the moisture content thereof to 15% to 25% uniformly distributed throughout the upper leather, lasting the upper while said upper is moist, heating the upper in a high temperature moist atmosphere having a dew point above the temperature of the upper prior to exposure thereto for a period sufficient to raise the temperature of the upper above the dew point of the atmosphere, said atmosphere being in the temperature range of 220° F. to 375° F., and thereafter drying the upper in said atmosphere.

#### References Cited by the Examiner

#### UNITED STATES PATENTS

45 2,973,530 3/61 Bromfield ----- 12—142

JORDAN FRANKLIN, Primary Examiner.